

# United States Patent Office

2,843,513

Patented July 15, 1958

1

2,843,513

## MIXTURE AND METHOD FOR IMPARTING A CORROSION-RESISTANT SURFACE TO ALUMINUM, ALUMINUM ALLOYS, AND SILVER

Raymond Stricklen, Baltimore, Md., assignor to Allied Research Products, Inc., Baltimore, Md., a corporation of Maryland

No Drawing. Application July 28, 1954  
Serial No. 446,407

21 Claims. (Cl. 148—6.2)

This invention relates to the treatment of aluminum, alloys wherein aluminum is the primary constituent and to silver. Aluminum is provided with a corrosion resistant chromate conversion coating which has additional characteristics to be listed hereinafter. Silver is provided with a tarnish resistant coating which will also be described in detail.

This application is a continuation-in-part of applicant's co-pending application, Serial No. 295,552, filed June 25, 1952, now abandoned, the latter being a continuation-in-part of applicant's application Serial No. 139,114, filed January 17, 1950, now abandoned.

In the case of aluminum, the coatings previously used commercially have been anodic oxide films produced by electrolysis in acid or alkaline solutions; oxide films produced chemically in alkaline oxidizing solutions; and phosphate coatings produced in acid phosphate solutions which may or may not have been modified by the presence of chromates.

The present invention provides equal or superior corrosion resistance to any of the above. It removes the necessity of high solution temperature and ventilation required in all of these prior treatment methods. It shortens the immersion time necessary to reach an equal degree of protection. It removes the necessity for power supply and the individual racking of parts necessary in the anodic processes. Furthermore, it is equally applicable to all alloys of aluminum in common use while the widely used chromic acid anodizing process is limited to those which contain 4.5% or less of copper.

An additional advantage is the fact that all of the coatings of those processes previously used are electrical insulators while those obtained through this invention are electrical conductors. The electrical resistance of the present coatings is on the order of 1900 microhms per square inch at a pressure of 100 pounds per square inch which is negligible for most purposes. This has enabled manufacturers of electrical equipment to protect aluminum surfaces from corrosion and to make electrical contact with the same surfaces without removing the protective coating. Results include lowered manufacturing costs and new flexibility of design possibilities.

The coating of the present invention has also been found advantageous in preparing aluminum for assembly by means of structural adhesives and has proved successful in bonding rubber to aluminum surfaces. In addition, it has been found to produce exceptionally durable bonds for paints and similar organic finishes.

In the assembly of aluminum parts by the inert gas shielded arc welding method it was previously necessary to weld immediately after mechanical or chemical cleaning of the metal. A delay of as much as 24 hours allows reformation of the natural oxides on the aluminum and these interfere with obtaining optimum weld characteristics. When the aluminum parts are treated by this invention after cleaning, they may be stored as long as several months and may still be welded without removal of the coating or without further cleaning. Further-

2

more, the welds produced in metal treated by this invention are found to be of superior quality. This property enables manufacturers to operate separate schedules for their cleaning and welding operations and to make use of smaller equipment than would be necessary for treating completed assemblies. After welding the weld beads are cleaned by wire brushing or equivalent and then treated by brush application of the solutions described in this invention, thereby providing protection for the entire assembly.

A further property of the coatings of this invention is their ability to absorb dyes. While still wet, the coatings are immersed in a solution of an organic dye and thereby colored in a manner permitting ready identification in color code systems and the like.

Aluminum alloys treated with the solutions of this invention for a period of 10 to 30 seconds are coated with a clear invisible film having appreciable corrosion protection. The protection is apparent on subjecting treated and untreated specimens to corrosive conditions such as the salt spray test described in Federal specification QQ-M-151. This is the first commercial process of the chemical immersion type to produce this type of protective clear film on alloys containing a high percentage of silicon.

Treatment of 30 seconds or more produces a yellow to light brown film which may exhibit considerable iridescence. Immersion in the range of 3 to 6 minutes produces films of a thickness suitable for coloring by dyes. The treatment time may be extended to ten minutes, however, some softness and powderiness may appear when the treatment exceeds six minutes. Although this has no adverse effect on corrosion protection, the appearance may be undesirable for some applications. The film formed by this process also exhibits the self-healing characteristics of other chromate films in protecting abraded areas.

Regarding silver and alloys containing silver as a primary constituent, an immersion of 10 seconds to 2 minutes produces a film of a pale yellow color which is barely visible. It is difficult to see under some conditions unless a treated piece is compared directly with an untreated piece.

The coating attained on silver has a high degree of tarnish resistance, being comparable with water dip lacquers which are widely used in tarnish protection on silver plate for industrial applications.

Its electrical contact resistance is on the order of 60 to 100 microhms per square inch of surface under a pressure of 100 pounds per square inch. This value is said to be negligible for most applications.

Silver surfaces which have been treated remain solderable under conditions which would tarnish untreated silver to such an extent that soldering is prevented.

The invention may comprise an acid chromate solution or a dry powder mixture which may be dissolved in water to form such a solution. The solution may contain chromic acid 1 to 15 grams per liter, sodium fluosilicate (silicofluoride) 5 grams per liter to 25 grams per liter or to saturation whichever is lower and boric acid 1 gram per liter to 45 grams per liter or to saturation, whichever is lower. The saturation concentrations of the sodium fluosilicate and the boric acid depend on the operating temperature and the pH selected. An excess of either compound remains on the bottom of the container, undissolved and has no effect on the reaction. A large excess of undissolved materials would be avoided in practice for reasons of economy.

When the solution is prepared from a supply of water which is nearly neutral (pH 5.5 to 7.5) the pH value of the solution will be well on the acid side, namely not above pH 4.0 and usually between about pH 2.5 to pH 1.3.

A lower limit of pH 0.8 is contemplated but not preferred. If the pH of the solution is not below 2.3, small quantities of a mineral acid, preferably nitric, are added to adjust the pH. Other mineral acids that may be used include any of the commercial grades of sulfuric, chromic, fluosilicic and fluoboric acid. In operation, the solution is maintained at the selected concentration, preferably by adding a suitable mixture of dry powdered materials, and sufficient mineral acid to maintain the pH within the selected range.

The preferred solutions will fall within the following ranges:

|                                  | G./l.     |
|----------------------------------|-----------|
| CrO <sub>3</sub>                 | 2.5 to 7  |
| Na <sub>2</sub> SiF <sub>6</sub> | 4.0 to 12 |
| H <sub>3</sub> BO <sub>3</sub>   | 4.0 to 12 |

and are made by dissolving a mixture of dry powdered materials in water. The dry powdered mixture is used primarily for its low cost in packaging and shipping although a liquid concentrate could be prepared which would serve the purpose.

The preferred dry mixture is as follows:

|                                  | Percent by weight |
|----------------------------------|-------------------|
| CrO <sub>3</sub>                 | 23                |
| Na <sub>2</sub> SiF <sub>6</sub> | 38.5              |
| H <sub>3</sub> BO <sub>3</sub>   | 38.5              |

It may be dissolved in a concentration between 10 and 85 g./l. of solution. A solution of about 22.5 g./l. (3.0 oz./gal.) gives a solution of the following composition.

#### Example I

|                                  | G./l. |
|----------------------------------|-------|
| CrO <sub>3</sub>                 | 5.2   |
| Na <sub>2</sub> SiF <sub>6</sub> | 8.65  |
| H <sub>3</sub> BO <sub>3</sub>   | 8.65  |

A solution with a pH of about 1.6 is generally obtained. If the pH is above 1.8 it is lowered by small additions of chromic, fluosilicic, fluoboric, sulfuric, or nitric acids. The latter is preferred.

If the pH of the solution is below 1.5 it may act too rapidly for the mechanical limitations of the work handling facilities. If desired the pH may be raised by small additions of NaOH or NH<sub>4</sub>OH. Either is satisfactory. The pH is best measured by means of a glass electrode and electrometer. The concentration of the solution is determined by iodometric titration.

The solution of Example I is preferred for aluminum parts which are to be treated by immersion or by brushing; and for silver plated parts which are handled in bulk. The results obtained by utilizing the foregoing example were quite favorable and produced a corrosion-resistant coating on aluminum and a tarnish-resistant coating on silver, as fully discussed heretofore. The immersion time for the foregoing was about 10 seconds and the temperature was about 30° C. Of course, these conditions can be varied as noted in the specification.

#### Example II

This solution is made by dissolving the preferred powder mixture at a concentration of 11.25 g./l. (1.5 oz./gallon).

|                                  | G./l. |
|----------------------------------|-------|
| CrO <sub>3</sub>                 | 2.6   |
| Na <sub>2</sub> SiF <sub>6</sub> | 4.3   |
| H <sub>3</sub> BO <sub>3</sub>   | 4.3   |

The operating range of this solution is between pH 1.8 and pH 2.3 and may be adjusted as described under Example I. This solution is recommended for aluminum in cases where the operation must be slowed down, for example, in spray operation and when clear films must be produced by slow moving mechanical equipment. It may be used for rack plated or other individually handled silver work.

The effectiveness, on aluminum, of the solutions heretofore disclosed may be improved by the addition of an inorganic chloride. Sodium chloride is preferred for its low cost but ammonium chloride, potassium chloride, ferric chloride may be substituted in stoichiometrically equivalent concentrations.

#### Example III

A suitable working solution containing the preferred sodium chloride consists of:

|                                  | G./l. |
|----------------------------------|-------|
| CrO <sub>3</sub>                 | 4.9   |
| Na <sub>2</sub> SiF <sub>6</sub> | 8.1   |
| H <sub>3</sub> BO <sub>3</sub>   | 8.1   |
| NaCl                             | 3.9   |

The pH of such a solution is about 1.3. It may be adjusted as in previous examples.

Although the solution of Examples I and II give excellent results, on aluminum, the use of the solution of Example III, which includes sodium chloride, yields definite improvements. For example, the resistance of the films resulting from immersion in said solution, to salt spray is increased by 50% to 500%. In addition, it should be noted that the optimum pH range of the working solution is extended by the addition of the inorganic chloride from the previous pH 1.3 to pH 2.5 to a new range of pH 1.0 to pH 3.0. By working in the lower end of this new pH range (pH 1.0 to pH 1.3) the treatment time for a given degree of protection may be shortened by as much as 50 to 75% when compared to the time necessitated in the utilization of the chloride free solution. The temperature range when utilizing the solution of Example III is 20° C. to 35° C.

The concentrations of chromic acid, sodium fluosilicate (silicofluoride) and boric acid may be within the ranges noted heretofore. When sodium chloride is utilized, as in Example III, the concentration thereof may vary from 0.5 gram per liter to 10 grams per liter.

Instead of immersing the aluminum, aluminum alloy, or silver articles in the solution, other means of treatment may be used, e. g., spraying, flow coating or brushing the solution on the articles.

While chromic acid is preferred, water-soluble compounds of salts of chromic acid capable of liberating chromic acid in water, such as alkali metal bichromates, may be used to give an equivalent amount of chromic acid as recited. Likewise, instead of boric acid, water-soluble boric acid salts, e. g., alkali metal borates capable of supplying boric acid in water may be used in amount to provide boric acid in equivalent amount to that set forth. Also, instead of the fluo compounds mentioned, other water-soluble fluo compounds, e. g., alkali metal or ammonium fluosilicates and fluoborates may be used in amount to liberate an equivalent amount of fluosilicic or fluoboric acid as indicated above.

Of course, it can be appreciated that different concentration ranges than those noted heretofore would be applicable to the use of salts of chromic acid, salts of boric acid, and other water-soluble fluosilicates and fluoborates. These different concentration ranges can be calculated using the ranges noted heretofore with respect to chromic acid, boric acid and sodium fluosilicate. In other words, the calculations should be such that the same amount of hexavalent chromium, borate, and fluorine radical would be realized in the mixture being formed.

In addition, as stated above, instead of the sodium chloride mentioned in Example III, other water-soluble chlorides, e. g., potassium chloride, ammonium chloride, or ferric chloride may be substituted. Again, different concentration ranges than that noted for the sodium chloride would be applicable. In other words, equivalent amounts of these other chlorides may be used and calculations should be such that the same amount of

chloride radical would be realized in the mixture being formed.

Examples of solutions utilizing compounds other than the preferred compounds are hereinafter set forth. Results that were obtained compare favorably with the results of Example I.

*Example IV*

|                                | G./L. |
|--------------------------------|-------|
| CrO <sub>3</sub>               | 4.9   |
| NaBF <sub>4</sub>              | 16.7  |
| H <sub>3</sub> BO <sub>3</sub> | 8.3   |

The pH of this solution is about 1.6 adjusted if necessary by the acid additions described for Example I. Other conditions are as in Example I.

*Example V*

|                                                  | G./L. |
|--------------------------------------------------|-------|
| CrO <sub>3</sub>                                 | 6     |
| H <sub>3</sub> BO <sub>3</sub>                   | 10    |
| (NH <sub>4</sub> ) <sub>2</sub> SiF <sub>6</sub> | 15    |

*Example VI*

|                                 | G./L. |
|---------------------------------|-------|
| CrO <sub>3</sub>                | 6     |
| H <sub>3</sub> BO <sub>3</sub>  | 10    |
| K <sub>2</sub> SiF <sub>6</sub> | 5     |

*Example VII*

|                                       | G./L. |
|---------------------------------------|-------|
| CrO <sub>3</sub>                      | 6     |
| H <sub>3</sub> BO <sub>3</sub>        | 10    |
| MgSiF <sub>6</sub> ·6H <sub>2</sub> O | 40    |

*Example VIII*

|                                | G./L. |
|--------------------------------|-------|
| CrO <sub>3</sub>               | 6     |
| H <sub>3</sub> BO <sub>3</sub> | 10    |
| NaBF <sub>4</sub>              | 15    |

pH of solutions in Examples V-VIII was about 1.6. Other conditions were as noted in Example I.

*Example IX*

|                                                                   | G./L. |
|-------------------------------------------------------------------|-------|
| Na <sub>2</sub> Cr <sub>2</sub> O <sub>7</sub> ·2H <sub>2</sub> O | 9     |
| H <sub>3</sub> BO <sub>3</sub>                                    | 10    |
| Na <sub>2</sub> SiF <sub>6</sub>                                  | 10    |
| HNO <sub>3</sub> to adjust pH to 1.5.                             |       |

*Example X*

|                                                                   | G./L. |
|-------------------------------------------------------------------|-------|
| CrO <sub>3</sub>                                                  | 6     |
| Na <sub>2</sub> B <sub>4</sub> O <sub>7</sub> ·10H <sub>2</sub> O | 15    |
| Na <sub>2</sub> SiF <sub>6</sub>                                  | 10    |
| HNO <sub>3</sub> to adjust pH to 1.5.                             |       |

Other conditions of Examples IX and X were as in Example I.

The exact mechanism of the formation of the corrosion resistant film is obscure. However, I believe that the following functions are performed by the constituents.

(1) The chromic acid or equivalent compound serves to supply the hexavalent chromium necessary in film formation.

(2) The fluosilicate or fluoroborate serves to activate the metal surface and to dissolve a small amount of metal. The solution of the metal reduces and precipitates chromium on the metal surface in a gel structure.

(3) The boric acid or borates act as a buffer, primarily at the metal-solution interface. At the interface the pH of the solution is higher than that in the main body of the solution. This condition is necessary for the precipitation of the reduced chromium. It is in this range that the boric acid is most effective in controlling the acidity. This control has the effect of improving the hardness of the precipitated tri-valent chromium film.

(4) The chloride, when present, accelerates precipitation and increases the thickness of the deposited film.

The novel principles of this invention are broader than the specific embodiments recited above, and rather than unduly extend this disclosure by attempting to list all the numerous modifications which have been conceived and reduced to practice during the course of this development, these novel features are substantially defined in the following claims.

I claim:

1. A dry powder mixture for use in an aqueous solution to impart a corrosion resistant coating to metals, consisting essentially of a chromic compound selected from the group consisting of chromic acid and water soluble salts thereof, a boric compound selected from the group consisting of boric acid and water soluble salts thereof, and a fluo compound selected from the group consisting of water soluble fluosilicates and fluoroborates, said chromic compound in amount being equivalent to from about 1 to 15 grams of chromic acid per liter of solution, said boric compound in amount being equivalent to from about 1 to 45 grams of boric acid per liter of solution, and said fluo compound in amount being equivalent to from about 5 to 25 grams of sodium fluosilicate per liter of solution.

2. An aqueous acidic solution to impart a corrosion resistant coating to metals, consisting essentially of water, a chromic compound selected from the group consisting of chromic acid and water soluble salts thereof, a boric compound selected from the group consisting of boric acid and water soluble salts thereof, a fluo compound selected from the group consisting of water soluble fluosilicates and fluoroborates, and a mineral acid, said chromic compound in amount being equivalent to from about 1 to 15 grams of chromic acid per liter of solution, said boric compound in amount being equivalent to from about 1 to 45 grams of boric acid per liter of solution, said fluo compound in amount being equivalent to from about 5 to 25 grams of sodium fluosilicate per liter of solution, and the mineral acid being equivalent in amount to give the aqueous solution a pH not greater than 4.0 or lower than 0.8.

3. An aqueous solution according to claim 2 having a concentration of the constituents in amount of about 10 to 85 grams per liter.

4. The method of treating aluminum, aluminum alloys, and silver, to produce thereon a corrosion resistant coating which comprises subjecting the same to an aqueous acidic solution consisting essentially of water, a chromic compound selected from the group consisting of chromic acid and water soluble salts thereof, a boric compound selected from the group consisting of boric acid and water soluble salts thereof, and a fluo compound selected from the group consisting of water soluble fluosilicates and fluoroborates, said solution having a pH between about pH 3.0 and pH 1.3, and wherein the chromic compound is in amount equivalent to from about 1 to 15 grams of chromic acid per liter of solution, said boric compound in amount equivalent to from about 1 to 45 grams of boric acid per liter of solution, and said fluo compound in amount equivalent to from about 5 to 25 grams of sodium fluosilicate per liter of solution, and wherein the concentration of ingredients is from about 10 to 85 grams per liter, and wherein the treatment is conducted with the solution at a temperature of about 20° C. to 35° C. for from about 10 seconds up to about 10 minutes.

5. The method of treating aluminum, aluminum alloys, and silver to produce thereon a corrosion resistant coating which comprises subjecting the same to an aqueous acidic solution consisting essentially of water, a chromic compound selected from the group consisting of chromic acid and water soluble salts thereof, a boric compound selected from the group consisting of boric acid and water soluble salts thereof, and a fluo compound selected from the group consisting of water soluble fluosilicates and fluoroborates, said solution having a pH between about

1.3 and 3.0, and wherein the chromic compound is present in amount equivalent to from about 1 to 15 grams of chromic acid per liter of solution, said boric compound in amount equivalent to from about 1 to 45 grams of boric acid per liter of solution, and said fluo compound in amount equivalent to from about 5 to 25 grams of sodium fluosilicate per liter of solution, and wherein the concentration of ingredients is about 10 to 85 grams per liter and wherein the treatment is conducted with the solution at a temperature of about 20° C. to 35° C. for from about 10 seconds up to about 10 minutes, and wherein the said solution is adjusted with mineral acid to a pH not greater than about 3.0 or less than about 1.3.

6. A dry powder mixture for use in aqueous solution to impart a corrosion resistant coating to metal, consisting essentially of a chromic compound selected from the group consisting of chromic acid and water soluble salts thereof, a boric compound selected from the group consisting of boric acid and water soluble salts thereof, a fluo compound selected from the group consisting of water soluble fluosilicates and fluoborates, and an inorganic chloride selected from the group consisting of an alkali metal chloride, ammonium chloride and ferric chloride, said chromic compound and said fluo compound being present in coating-producing proportions.

7. A dry powder mixture according to claim 6 wherein said chromic compound is in amount equivalent to from about 1 to 15 grams of chromic acid per liter of solution, said boric compound in amount equivalent to from about 1 to 45 grams of boric acid per liter of solution, said fluo compound in amount equivalent to from about 5 to 25 grams of sodium fluosilicate per liter of solution, and the inorganic chloride in amount equivalent to from about 0.5 to 10 grams of sodium chloride per liter of solution.

8. A dry powder mixture according to claim 6 wherein said inorganic chloride is sodium chloride.

9. A dry powder mixture according to claim 6 wherein said inorganic chloride is potassium chloride.

10. A dry powder mixture according to claim 6 wherein said inorganic chloride is ammonium chloride.

11. A dry powder mixture according to claim 6 wherein said inorganic chloride is ferric chloride.

12. An aqueous acidic solution to impart a corrosion resistant coating to metals, consisting essentially of water, a chromic compound selected from the group consisting of chromic acid and water soluble salts thereof, a boric compound selected from the group consisting of boric acid and water soluble salts thereof, a fluo compound selected from the group consisting of water soluble fluosilicates and fluoborates, and an inorganic chloride selected from the group consisting of alkali metal chloride, ammonium chloride and ferric chloride, said chromic compound and said fluo compound being present in coating-producing proportions.

13. An aqueous acidic solution according to claim 12 wherein the chromic compound is in amount equivalent to from about 1 to 15 grams of chromic acid per liter of solution, said boric compound in amount equivalent to from about 1 to 45 grams of boric acid per liter of solution, said fluo compound in amount equivalent to from about 5 to 25 grams of sodium fluosilicate per liter of solution, and the inorganic chloride is present in amount equivalent to from about 0.5 to 10 grams of sodium chloride per liter of solution.

14. An aqueous acidic solution according to claim 12 having a concentration of constituents in amount of about 10 to 85 grams per liter of solution.

15. An aqueous acidic solution according to claim 12 including a mineral acid in amount to give the aqueous solution a pH not greater than about 3.0 or less than about 1.0.

16. The method of treating aluminum, aluminum alloys and silver, to produce thereon a corrosion resistant coating which comprises subjecting the same to an aqueous acidic solution consisting essentially of water, a chromic compound selected from the group consisting of chromic acid and water soluble salts thereof, a boric compound selected from the group consisting of boric acid and water soluble salts thereof, a fluo compound selected from the group consisting of water soluble fluosilicates and fluoborates, and an inorganic chloride selected from the group consisting of an alkali metal chloride, ammonium chloride and ferric chloride, said chromic compound and said fluo compound being present in coating-producing proportions.

17. A method according to claim 16 wherein the chromic compound is present in amount equivalent to from about 1 to 15 grams of chromic acid per liter of solution, said boric compound in amount equivalent to from about 1 to 45 grams of boric acid per liter of solution, said fluo compound in amount equivalent to from about 5 to 25 grams of sodium fluosilicate per liter of solution, and the inorganic chloride is present in amount equivalent to from about 0.5 to 10 grams of sodium chloride per liter of solution, and wherein the solution is adjusted with mineral acid to a pH not greater than about 3 or less than about pH 1.3.

18. A method according to claim 16 wherein the treatment is conducted with the solution at a temperature of about 20° C. to 35° C.

19. An aqueous acidic solution to impart a corrosion resistant coating to aluminum, aluminum alloys, and silver, consisting essentially of water, chromic acid, boric acid and sodium fluosilicate.

20. An aqueous acidic solution as claimed in claim 19 wherein said chromic acid is in amount of 5.2 grams per liter of solution, the boric acid in amount of 8.65 grams per liter of solution, and the fluosilicate in amount of 8.65 grams per liter of solution.

21. An aqueous acid bath for coating aluminum and alloys thereof in which aluminum is the predominant ingredient, of the type wherein the essential coating-producing ingredients are hexavalent chromium and a soluble fluorine-bearing compound in coating-producing proportions; containing, as an addition agent, a quantity of boron (calculated as boric acid) in excess of the amount required for reaction with all of the fluorine present.

#### 53 References Cited in the file of this patent

#### UNITED STATES PATENTS

|           |              |               |
|-----------|--------------|---------------|
| 2,114,151 | Romig        | Apr. 12, 1938 |
| 2,276,353 | Thompson     | Mar. 17, 1942 |
| 2,477,841 | Ward         | Aug. 2, 1949  |
| 2,507,956 | Bruno et al. | May 16, 1950  |

#### FOREIGN PATENTS

|    |         |         |             |
|----|---------|---------|-------------|
| 65 | 675,334 | Germany | May 6, 1939 |
|----|---------|---------|-------------|